

April 30, 1935.

J. E. SCHOPP

1,999,260

COATED PAPER AND PROCESS OF MANUFACTURE

Filed June 27, 1932



INVENTOR  
John E. Schopp  
Chappell & Earl  
ATTORNEYS

## UNITED STATES PATENT OFFICE

1,999,260

COATED PAPER AND PROCESS OF  
MANUFACTURE

John E. Schopp, Oak Park, Ill.

Application June 27, 1932, Serial No. 619,375

8 Claims. (Cl. 91—68)

The objects of this invention are:

First, to provide varnished paper labels or any varnished paper that is of a superior quality and can be manufactured very economically, and a process for making the same.

Second, to provide a coated paper suitable for varnishing and the process of making the same.

Third, to provide such a paper that is impervious to varnish and which will not change color when varnished.

Fourth, to provide such a paper that will not absorb ink or varnish that is applied thereto.

Objects pertaining to details and economies of my invention will definitely appear from the description to follow. The invention is defined in the claims.

The manner of carrying out my invention is clearly illustrated in the accompanying drawing, in which:

Fig. 1 shows diagrammatically apparatus for carrying out my new process and manufacturing my new product.

Fig. 1-A shows diagrammatically apparatus for varnishing sheets of my improved paper.

Fig. 2 shows diagrammatically a different type of apparatus for applying coating.

Fig. 3 shows diagrammatically a still different type of apparatus for applying coatings.

Heretofore, in order to make a paper suitable for varnishing, it has been necessary to use large quantities of casein or other adhesive and to use satin white which is more expensive than clay for the coating in order to make a paper of the class produced by my process. To make a paper that is the closest to my paper but which is unsatisfactory for the purpose, it is necessary to use as a coating about one hundred parts by weight of satin white to twenty-two to twenty-five parts by weight of casein. The usual clay sized paper in which seventeen parts by weight of casein and one hundred parts by weight of clay are used is not satisfactory. By means of my process I have succeeded in making a better sheet more economically by applying two separate coatings differing from one another in their nature.

In describing my invention I refer to a "fifteen pound coat". This is the usual paper terminology and indicates that the coating applied to the paper is of such weight that the coating applied to a ream of five hundreds sheets of paper twenty-five by thirty-eight inches weighs fifteen pounds. Those skilled in the art will understand this terminology without further explanation.

In my process I first coat the web of paper with a fifteen pound coating containing approximately

one hundred parts by weight of clay or other pigment, fifty-three parts by weight of water and approximately seven parts by weight of dry casein.

After this coating is applied in the conventional manner I partially dry the paper and then apply a two pound coating containing about five parts by weight of dry casein to one hundred parts by weight of water. The paper is then dried and after printing a coat of varnish is applied in any usual manner, such as by the use of a machine as illustrated in Fig. 1-A or by what is known as overlay varnishing, which is merely printing the varnish on the sheet with the usual printing process.

Paper coated in this way is a superior product for varnishing and is in much demand. The varnish is held up by the coating because of the layer of adhesive applied after the original coating, which makes the final coated paper practically impervious to varnish.

I am aware of the well known process of applying two like coatings to a sheet and know that such processes do not embody the advantages of my process or produce my product.

Referring to the drawing, my process in detail is as follows:

1 is a roll of paper which is preferably a hard-sized paper, which I have found gives better results, although a soft-sized or unsized paper can be treated by my process. 2 is a coating applying machine comprising a color pan 3 and brass rolls 4 and 5 through which the web 6 of paper passes. The lower roll 5 picks up the pigment from the color pan and applies it to the face of the paper web 6, and the roll 4 is so positioned that it presses the paper and regulates the amount of coating applied to the paper. The device is conventional and is illustrated only diagrammatically.

The paper web 6 then passes over endless rubber apron 7 running over rolls 8 where oscillating brushes 9 spread out the coating. The paper is fed along by means of perforated rubber blanket 10 having a suction means therein. The means illustrated are all conventional and are illustrated diagrammatically.

In carrying out my process, in color pan 3 I place a coating composition made up of one hundred parts by weight of clay, fifty-three parts by weight of water and fifty parts by weight of casein solution. Fifty parts of casein solution is equal to about seven parts dry casein, and the solution herein referred to is made up of one hundred parts by weight of casein, six hundred parts by weight of water and five parts by weight of soda ash.

It may be necessary, depending upon the sizing of the paper, to use more or less casein, but it will be approximately in the proportions set forth.

5 Although I have described the use of casein, clay and soda ash, I do not wish to be limited to these products alone because I have found that my process works equally well if instead of clay, I use satin white, blanc fixe, calcium carbonate, 10 natural calcium sulphate, or any other pigment that may be used in the coating of paper. Instead of casein it is possible to use any adhesive used in coating paper or suitable for such use, such as starch or glue, and I do not wish to be limited to the use of casein alone, although it is the best adhesive now available. It is also possible to use any suitable alkali instead of soda ash in making the casein solution. The various 15 pigments can be blended as desired and the adhesives can also be blended to obtain desired results.

After the paper has passed the suction apron 10 it is festooned over sticks 11 for drying. At this point in carrying out my process, I dry the 20 paper until it is partially dry. I prefer to leave about fifteen to twenty per cent of moisture in the paper, but this can be varied. I have illustrated the drying as by festooning the paper, which is well known in the trade. It may also 25 be dried by steam coils or blasts of heated air may be blown upon the paper, the only requisite being that the paper be dried.

The paper passes from the drying to a series of wooden rolls 12 which are conventional and 30 smooth out any wrinkles in the web.

35 The web passes then to a second coating applying apparatus 13 similar in all respects to the apparatus 2. The coating is then treated as before by oscillating brushes 14 and the web is fed along by suction apron 15 similar to suction apron 10. The paper is then festooned on sticks 16 and dried, as is well known in the art, and passes over a metal guide 17 through smoothing rolls 18 where it is wound on storage roll 19.

40 In the apparatus 13 I apply a coating different from that applied in the machine 2. I apply a two pound coating. To apply this coating I use a solution comprising thirty-five parts by weight of casein solution such as heretofore described, or about five parts by weight of dry casein to 45 one hundred parts by weight of water in the apparatus 13. The coating is applied as before and the steps of treatment above outlined are followed. Instead of casein, any desired adhesive, as stated above, can be used, and it is not 50 necessary to use casein in the apparatus 2 and also in the apparatus 13. Any desired adhesive may be used in either apparatus without departing from my invention.

55 The proportions of materials may be varied but they need never be raised to the quantities required by the former treatment. In manufacturing my product, I have referred to applying a fifteen pound coating to the paper and then 60 applying a two pound coating of the adhesive. My invention can be used in varying proportions, and I have found that the second coating, to-wit, the adhesive, can be as light as or lighter than one pound. The proportions by weight of the 65 pigment for the first coating may vary considerably from the ratio heretofore described. These factors are dependent upon the sizing of the paper to be coated and its absorptive qualities.

70 75 I have described the production of a seventeen

75 pound coating. For heavier coatings a heavier coat is put on the paper in the first instance and the second coating may be as described or of a different weight, depending upon the conditions. The first coating is usually one that will 80 stick to the paper but is not a coating that in and of itself would be sufficient, although I have found that a much better sheet of paper can be made if a coating that was heretofore considered satisfactory is given a light second coat of 85 adhesive.

90 The paper produced is coated by a bound coating of the clay with a thin overlaid film of the adhesive alone, which makes the paper impervious to varnish or ink.

95 In Fig. 2 I illustrate an apparatus 20 for use in place of either the apparatus 2 or 13. This apparatus has a color pan 21, brass roller 22, brush 23 for applying the coating to the web 6 as it is carried around a bras roll 24.

100 In Fig. 3 is an apparatus 25 that can be used in place of apparatus 2 or apparatus 13, or apparatus 20. A color tank 26 is provided with brass rolls 27 and 28 through which the web 6 of paper passes. Nozzle 29 discharges the coating on the 105 sheet and the rolls 27 and 28 squeeze it to regulate the quantity applied.

110 In Fig. 1-A I show apparatus suitable for applying varnish to my paper. The varnish can be applied immediately after the paper is completed. This is not done if the paper is to be 115 printed for labels because a varnished sheet will not take ink and the printing would not be protected by the varnish. The apparatus shown is for use in applying spirit varnish to printed labels 120 or other sheets.

125 The sheets 30 are fed between rubber roll 31 and brass roll 32. The rubber roll 31 applies varnish taken up by brass roll 33 from tank 34. The labels 30 are then fed to a continuous conveyor 35 which passes beneath suitable drying means 36, here illustrated as a hood with suitable inlets 37 for heated air. The labels are fed through the 130 drying apparatus and are stacked as shown at 38. The varnish used is a copal gum and denatured 135 alcohol solution. Other varnishes may be applied and the varnish may be applied by printing, which is known as overlay varnish.

140 The paper produced in this manner may be produced for wall paper as well as labels and is 145 suitable for any use wherein a waterproof paper is desired.

150 Modifications of my process can be utilized for making a paper that is very resistant to ink and the quantities of materials used may be lowered 155 considerably and the paper thus treated will, although not suitable for varnish, be suitable for printing and be a superior product.

Having thus described my invention, what I claim as new and desire to secure by Letters 160 Patent is:

1. The method of making varnished paper comprising coating the paper with a mixture of pigment and casein in which the quantity of casein is sufficient to hold the pigment to the paper during manipulation of the paper in coating but is not sufficient to permanently hold the pigment to the paper, drying said coating, applying a second coating of from approximately 1 to approximately 2 pounds in weight comprising casein only, drying 165 said second coating and applying a coat of varnish.

2. The method of making paper for printing comprising coating the paper with a mixture of pigment and casein in which the quantity of 170

casein is sufficient to hold the pigment to the paper during manipulation of the paper in coating but is not sufficient to permanently hold the pigment to the paper, drying said coating and applying a second coating of from approximately 1 to approximately 2 pounds in weight comprising casein only.

3. The method of making paper for printing comprising coating the paper with a mixture of 10 pigment and an adhesive selected from the class consisting of glue, starch and casein, in which the quantity of said adhesive is sufficient to hold the pigment to the paper during manipulation of the paper in coating but is not sufficient to permanently hold the pigment to the paper, drying said coating, applying a second coating of from approximately 1 to approximately 2 pounds in weight comprising said adhesive only.

4. The method of making paper for printing comprising coating paper with a coating having therein approximately 100 parts by weight of pigment to 7 parts by weight of casein, drying said coating and then applying thereto a coating of casein of from approximately 1 to approximately 2 pounds in weight.

5. An article of manufacture comprising a sheet of paper made by coating the paper with a mixture of pigment and casein in which the quantity of casein is sufficient to hold the pigment to the paper during manipulation of the paper in coating but is not sufficient to permanently hold the pigment to the paper, drying said coating, applying a second coating of from approximately 1 to

approximately 2 pounds in weight, comprising casein only, drying said second coating and applying a coat of varnish.

6. An article of manufacture comprising a sheet of paper made by coating the paper with a mixture of pigment and casein in which the quantity of casein is sufficient to hold the pigment to the paper during manipulation of the paper in coating but is not sufficient to permanently hold the pigment to the paper, drying said coating and applying a second coating of from approximately 1 to approximately 2 pounds in weight comprising casein only.

7. An article of manufacture comprising a sheet of paper made by coating the paper with a mixture of pigment and an adhesive selected from the class consisting of glue, starch and casein, in which the quantity of said adhesive is sufficient to hold the pigment to the paper during manipulation of the paper in coating but is not sufficient to permanently hold the pigment to the paper, drying said coating, applying a second coating of from approximately 1 to approximately 2 pounds in weight comprising said adhesive only.

8. An article of manufacture comprising a sheet of paper made by coating paper with a coating having therein approximately 100 parts by weight of pigment to 7 parts by weight of casein, drying said coating and then applying thereto a coating of casein of from approximately 1 to approximately 2 pounds in weight.

JOHN E. SCHOPP.